

May 25, 1954

H. D. NORRIS ET AL

2,679,481

ANTIOXIDANTS

Filed Feb. 7, 1952



INVENTORS  
HENRY D. NORRIS  
RALPH V. WHITE  
BY

*Hastings S. Trigg*

AGENT

## UNITED STATES PATENT OFFICE

2,679,481

## ANTIOXIDANTS

Henry D. Norris, Woodbury, and Ralph V. White,  
Pitman, N. J., assignors to Socony-Vacuum Oil  
Company, Incorporated, a corporation of New  
York

Application February 7, 1952, Serial No. 270,303

7 Claims. (Cl. 252—50)

1

This invention relates, broadly, to lubricants containing organic nitrogen compounds. It is more specifically concerned with mineral lubricating oils having improved resistance to oxidation.

As is well known to those skilled in the art, most lubricants undergo a relatively rapid deterioration during use, as the result of the effects of oxidation. This oxidation is effected by a combination of factors, including relatively high temperatures and atmospheric oxygen. It is hastened, i. e., catalyzed, by metals, such as iron, copper, and copper alloys, which are present in lubrication systems. Oxidation of a lubricating oil is manifested by the formation of corrosive, acidic bodies, sludge, and high color. Especially highly refined lubricating oils, such as those used for lubricating steam turbines, are particularly susceptible to oxidation. That such action, together with its undesirable manifestations, cannot be tolerated in such engines, will be readily appreciated by those skilled in the art.

It has now been found that certain nitrogen-containing organic compounds effectively inhibit the oxidation of lubricants. It has now been discovered that mineral lubricating oils containing specific piperazine compounds are resistant to oxidation. In U. S. Patent No. 2,816,587, the use of diaryl piperazines to stabilize transformer oils is proposed. It has been found, however, that these compounds are not effective in the present invention, and are not contemplated within the scope of this invention.

Accordingly, it is a broad object of the present invention to provide lubricants having increased resistance to oxidation. Another object is to provide improved mineral lubricating oils containing organic nitrogen-containing compounds. A specific object is to provide mineral lubricating oils containing specific piperazine compounds, which oils have an increased resistance to oxidation. Other objects and advantages of this invention will become apparent to those skilled in the art, from the following detailed description.

The present invention provides a mineral lubricating oil containing a small amount, sufficient to stabilize it against oxidation, of a com-

2

pound selected from the group consisting of (1) compounds having the formula,



wherein R is a radical of the group consisting of  $\beta$ -(phenylamino)ethyl,  $\beta$ -(naphthylamino)ethyl,  $\beta$ -(o-tolylamino)ethyl, and  $\beta$ -(m-tolylamino)ethyl radicals, and Y is a radical of the group consisting of phenyl, naphthyl, o-tolyl, and m-tolyl radicals; and (2) compounds having the formula,



wherein  $\text{R}''$  is an alkyl radical having between one and 8 carbon atoms, and  $\text{R}'$  is a radical of the group consisting of phenyl and naphthyl radicals and the radical having the formula,



The compounds having the formula,



wherein R and Y are as set forth hereinbefore, is readily prepared by reacting a primary aryl amine with a tri-( $\beta$ -haloethyl) amine hydrohalide with the elimination of hydrogen halide.

35 The halogen thereof can be chloro, bromo, or iodo. The aryl amine is reacted with the trihaloethylamine hydrohalide reactant in a molar proportion of 2:1, respectively. The following equation illustrates the reaction involved, with aniline used as the aryl amine reactant:



In order to produce compounds which are ef-

fective in this invention, the arylamine reactant must be aniline, naphthylamine, o-toluidine, or m-toluidine. It has been found that alkyl or aryl substituents on the aromatic ring generally detract from the antioxidant properties of the compounds derived therefrom. Exceptions to this general rule occur in the case of o- and m-toluidines. Other ring-alkylated aromatic primary amines and even p-toluidine produce compounds which have little antioxidant properties when blended in a lubricating oil. In fact, many are pro-oxidants. Other substituents, such as nitro, hydroxyl, alkoxy, and the like radicals, also, have an adverse effect upon the antioxidant properties of the compounds contemplated herein.

The compounds having the formula,



wherein R' and R'' are as aforescribed, are prepared by reacting a primary arylamine with a di( $\beta$ -haloethyl)alkylamine hydrohalide in a molar proportion of 1:1, respectively. As illustrated with aniline and di-(bromoethyl)methylamine hydrobromide, the reaction proceeds in accordance with the equation:



The di-( $\beta$ -haloethyl)alkylamine hydrohalide reactant can contain between one and 8 carbon atoms per alkyl radical. The halogen atoms thereof can be bromo, chloro, or iodo atoms. Non-limiting examples of the alkyl radicals of these amines, which radicals can be straight-chain or branched-chain, are methyl, propyl, isopropyl, ethyl, butyl, isobutyl, t-butyl, amyl, sec-amyl, hexyl, isoheptyl, octyl, and 2-ethylhexyl radicals. The primary aromatic amines which react with the dihaloethylalkylamine reactant, as aforescribed, to form the additives of type (2) are aniline, naphthylamine, and 4,4'-diaminodiphenylmethane. Since there are two amino groups in the latter amine which can react, the additive compound is prepared by reacting two moles of di-( $\beta$ -haloethyl)alkylamine with each mole of 4,4'-diaminodiphenylmethane. As is the case of the aromatic amine reactants in Equation 1, these aromatic amines cannot have other substituent groups on the aromatic ring, without detracting from the anti-oxidant properties of the compounds produced therefrom. In the compounds illustrated by Equation 2, whenever there is an aryl group attached directly to one nitrogen atom of piperazine, there must be an alkyl group of one to 8 carbon atoms attached to the other. In other words, diarylpiperazines are not effective in the present invention.

In both reactions illustrated by the Equations 1 and 2, it will be noted that hydrogen halide is a by-product of the reaction. In order to ensure complete reaction, in accordance with the principle of Le Chatelier, the hydrogen halide should be removed or chemically immobilized. This can be effected by having sufficient hydrogen halide acceptor present in the reaction system to combine with the hydrogen halide. Amines are often used for this purpose, forming the amine hydrohalide. This amine can be an excessive

amount of the aromatic amine reactant, or it can be another amine, preferably a tertiary alkylamine. Thus, in Equation 1, six moles of aniline could be used, i. e., two moles for the principal reaction and four moles to react with the hydrogen halide. Alternatively, at least four equivalents of a suitable hydrogen halide acceptor can be used. Suitable hydrogen halide acceptors include trialkylamines (tributylamine, triamylamine, triethylamine, etc.), heterocyclic nitrogen compounds (pyridine, piperidine, etc.), inorganic bases (sodium carbonate, sodium bicarbonate, etc.), and many others well known to those skilled in the art.

The compounds utilized in this invention are prepared at temperatures of between about 160° C. and about 240° C., preferably between about 200° C. and about 230° C. The time of reaction varies, dependent on the temperature and the reactants involved, between about three hours and about 15 hours. Product separation can be effected by usual methods, including distilling and/or filtering off excess reactants and amine hydrohalide. The residue is the desired compound in a substantially pure form. This can be subjected to further purification steps well known to the art, e. g., extraction or crystallization.

The piperazine compounds utilizable for the purposes of the present invention are blended in a mineral lubricating oil at concentrations of between about 0.05 per cent, by weight, and about 5 per cent, by weight. Preferably the concentration varies between about 0.1 per cent and about 2 per cent. Mineral oil concentrates of the additive compounds are contemplated. Thus, more than 5 per cent, by weight, and up to about 49 per cent of the additive (limited by the dispersibility thereof in mineral oil) could be blended in a mineral oil fraction. The resultant concentrate can be diluted, at any time prior to use, with a suitable amount of the mineral lubricating oil to be inhibited, thereby achieving, ultimately, a mineral oil blend containing the desired amount of additive.

The following specific working examples are for the purpose of illustrating the additives contemplated herein and to demonstrate their effectiveness. This invention is not to be limited to the specific compounds used, or to the operations and manipulations involved therein. Other compounds, as described hereinbefore, can be used, as those familiar with the art will readily understand.

#### EFFECTIVE COMPOUNDS

Example 1.—N-[ $\beta$ -(anilino)ethyl]-N'-phenylpiperazine

Tri-( $\beta$ -chloroethyl)amine hydrochloride (15 grams, 0.062 mole) and aniline (45 grams, 0.484 mole) were placed in a reaction vessel and heated at reflux temperatures for 3 hours. During the reflux period, the temperature of the reaction mixture rose from 185° C. to 210° C. The reaction mixture was cooled and made strongly basic with 250 milliliters of a 10-per cent, by weight, aqueous sodium hydroxide solution. Then, the mixture was steam distilled until 100 milliliters of distillate showed no appreciable amount of aniline distilling. The residual product was cooled and taken up with 250 milliliters of diethyl ether. The ether solution was washed with water and dried over solid potassium hydroxide. The solution was filtered, and the ether was removed by evaporation over the steam bath, leaving 18

grams of oily product. After this oil stood for a few days, crystals appeared. These were recrystallized from dilute alcohol, and were found to have a melting point of 58-59° C. In Rec. Trav. Chim., 56, 1007 (1937), van Alphen reported a melting point of 60° C. for the product of this example, i. e., N-[ $\beta$ -(anilino)-ethyl]-N'-phenylpiperazine.

*Example 2.—N-[ $\beta$ -(1-naphthylamino)ethyl]-N'-1-naphthylpiperazine*

Tri-( $\beta$ -chloroethyl) amine hydrochloride (12.05 grams, 0.05 mole), 1-naphthylamine (14.3 grams, one mole), and tri-n-butylamine (46.2 grams, 0.25 mole) were placed in a reaction vessel and refluxed for 6 hours at 216° C. The reaction mixture was cooled, and made distinctly alkaline with about 250 milliliters of a 10 per cent, by weight, aqueous solution of sodium hydroxide. The mixture was subjected to steam distillation until all of the tri-n-butylamine had been distilled out. The residual material was taken up in diethyl ether (about 250 milliliters) and washed with water. The ethereal solution was dried over solid potassium hydroxide and filtered. The ether was evaporated from the filtrate, over the steam bath. The product (19 grams thereof) was a dark-colored oil which contained no halogen, and 9.67 per cent nitrogen.

*Example 3.—N-(1-naphthyl)-N'-n-butylpiperazine*

N,N-di( $\beta$ -chloroethyl)-n-butylamine hydrochloride, 1-naphthylamine, and tri-n-butylamine, in a molar proportion of 1:1:3.3, respectively, were heated together at 210° C. for four hours. N-(1-naphthyl)-N'-n-butylpiperazine was obtained from the reaction mixture in accordance with the method set forth in Example 2. The isolated product contained 9.1 per cent nitrogen.

*Example 4.—N-phenyl-N'-n-butylpiperazine*

Aniline and N,N-di( $\beta$ -chloroethyl)-n-butylamine hydrochloride, in a molar proportion of 5:1, respectively, were reacted at 210° C. for 3.5 hours. N-phenyl-N'-n-butylpiperazine, containing 12.89 per cent nitrogen, was isolated as described in Example 1.

*Example 5.—4,4'-di[1-(4-n-butylpiperazino)]diphenylmethane*

N,N-di( $\beta$ -chloroethyl)-n-butylamine hydrochloride, 4,4'-diaminodiphenylmethane, and tri-n-butylamine, in a molar proportion of 2:1:7, respectively, were refluxed together at 216° C. for 9 hours. The product, containing 11.16 per cent nitrogen, was isolated in accordance with the procedure set forth in Example 2. This compound has the structural formula:



*Example 6.—N-[ $\beta$ -(m-tolylamino)ethyl]-N'-m-tolylpiperazine*

Tri-( $\beta$ -chloroethyl) amine hydrochloride, m-toluidine, and tri-n-butylamine, in a molar proportion of 1:2:4.5, respectively, were heated in a closed bomb for 12 hours at 230° C. N-[ $\beta$ -(m-tolylamino)ethyl]-N'-m-tolylpiperazine was obtained therefrom, in accordance with the procedure described in Example 2.

*Example 7.—N-[ $\beta$ -(o-tolylamino)ethyl]-N'-o-tolylpiperazine*

Tri-( $\beta$ -chloroethyl) amine hydrochloride, o-tolu-

idine, and tri-n-butylamine, in a molar proportion of 1:2:4.5, respectively, were heated in a closed bomb at 230° C. for 12 hours. N-[ $\beta$ -(o-tolylamino)ethyl]-N'-o-tolylpiperazine was obtained therefrom, in accordance with the procedure described in Example 2.

#### INEFFECTIVE COMPOUNDS

The following substituted piperazines were found to be ineffective for the purposes of this invention.

*Examples 8 and 9.—N-[ $\beta$ -(p-t-amylphenylamino)ethyl]-N'-(p-t-amylphenyl)piperazine*

Tri-( $\beta$ -chloroethyl) amine hydrochloride, p-t-amylaniline, and tri-n-butylamine, in a molar proportion of 1:2:5, respectively, were heated together at 210° C. for 8 hours. Using the method of Example 2, N-[ $\beta$ -(p-t-amylphenylamino)ethyl]-N'-(p-t-amylphenyl)piperazine was obtained from this reaction. In a second preparation, the same reactants in the same proportions were heated in a closed bomb for 12 hours at 230° C. The product was isolated as aforescribed.

*Example 10.—N-[ $\beta$ -(p-tolylamino)ethyl]-N'-p-tolylpiperazine*

Tri-( $\beta$ -chloroethyl) amine hydrochloride, p-toluidine, and tri-n-butylamine, in a molar proportion of 1:2:4.5, were heated together in a closed bomb for 12 hours at 230° C. The product, N-[ $\beta$ -(p-tolylamino)ethyl]-N'-p-tolylpiperazine, was isolated using the method described in Example 2.

*Example 11.—N,N'-diphenylpiperazine*

This compound was prepared by reacting aniline with ethylene bromide, in a molar proportion of 1:1.3, respectively, for 4 hours at 160° C.

*Example 12.—N,N'-di(p-t-amylphenyl)piperazine*

This compound was obtained from the reaction of p-t-amylaniline, ethylene bromide, and sodium carbonate, in a molar proportion of 1:1:1, respectively, at 160° C., for 7 hours.

#### TEST DATA

The base oil used in testing the aforescribed compounds is a furfural refined Midcontinent (Rodessa) distillate stock. It has a specific gravity of 0.860, a flash point of 405° F., and a viscosity of 155 S. S. U. at 100° F. This oil is suited for use in steam turbines.

*Example 13*

Each of the products of Examples 1 through 12 was blended in portions of the base oil at a concentration of 0.2 per cent, by weight. Each blend was subjected to the Brown-Boveri Turbine Oil Test. This test is described in the Brown-Boveri Rev., 16 (2), 92-7 (1929). Briefly, a 200-milliliter sample of oil under test is placed in a 400-milliliter covered beaker containing a V-shaped piece of polished copper. Air is passed over the surface of the oil at a rate of two liters per hour. The test is conducted for 72 hours at 230° C. and then for 24 hours at room temperature. The results, in terms of condition of the copper, neutralization number (N.N.), and Lovibond color, indicate the oxidation stability of the oil. These results are compared with similar results for the uninhibited base oil. Pertinent test data for compounds of Examples 1 through 7 are set forth in Table I. Similar data for the

7  
ineffective compounds of Examples 8 through 12 are set forth in Table II.

Table I.—Brown-Boveri Turbine Oil Test  
EFFECTIVE COMPOUNDS BLENDED AT 0.2% CONCENTRATION IN OIL

| Example | Compound Tested                                                            | Color, Lovibond | N. N.*       | Copper         | 5  |
|---------|----------------------------------------------------------------------------|-----------------|--------------|----------------|----|
| 1.      | Uninhibited Base Oil—<br>N-[ $\beta$ -(anilino)ethyl]-N'-phenylpiperazine. | 58<br>1.1       | 0.19<br>0.01 | O. K.<br>O. K. | 10 |
| 2.      | N-[ $\beta$ -(1-naphthylamino)ethyl]-N'-(1-naphthyl)piperazine.            | 3.2             | 0.02         | O. K.          | 4  |
| 3.      | N-(1-naphthyl)-N'-n-butylpiperazine.                                       | 6.0             | 0.02         | O. K.          | 15 |
| 4.      | N-phenyl-N'-n-butylpiperazine.                                             | 1.5             | 0.02         | O. K.          | 5  |
| 5.      | 4,4'-di[1-(4-n-butylpiperazino)]diphenylmethane.                           | 1.3             | 0.01         | O. K.          | 12 |
| 6.      | N-[ $\beta$ -(m-tolylamino)ethyl]-N'-m-tolylpiperazine.                    | 1.5             | 0.03         | O. K.          | 20 |
| 7.      | N-[ $\beta$ -(o-tolylamino)ethyl]-N'-o-tolylpiperazine.                    | 1.5             | 0.03         | O. K.          |    |

\*Neutralization number.

Table II.—Brown-Boveri Turbine Oil Test  
INEFFECTIVE COMPOUNDS BLENDED AT 0.2% CONCENTRATION IN OIL

| Example | Compound Tested                                                                                 | Color, Lovibond | N. N.*       | Copper           | 30 |
|---------|-------------------------------------------------------------------------------------------------|-----------------|--------------|------------------|----|
| 8.      | Uninhibited Base Oil—<br>N-[ $\beta$ -(p-t-amylphenylamino)-ethyl]-N'-p-t-amylphenylpiperazine. | 58<br>58        | 0.19<br>0.70 | O. K.<br>Bright. |    |
| 9.      | do                                                                                              | 65              | 0.65         | Do.              | 35 |
| 10.     | N-[ $\beta$ -(p-tolylamino)ethyl]-N'-p-tolylpiperazine.                                         | 6               | 0.15         | O. K.            |    |
| 11.     | N,N'-diphenylpiperazine.                                                                        | 7               | 0.89         | O. K.            | 40 |
| 12.     | N,N'-di(p-t-amylphenyl)piperazine.                                                              | 9               | 0.10         | O. K.            |    |

\* Neutralization number.

Example 14

Some of the reaction products described in the preceding examples were subjected to the ASTM Turbine Oil Oxidation Test. This test is fully described in the ASTM Manual, as Test D-943-47T. In general, the test involves placing a 300-milliliter sample of test oil in a tube provided with a gas inlet having a fritted glass outlet, and a catalyst coil consisting of interwound iron and copper wire. The test is conducted at a temperature of  $203 \pm 0.9^{\circ}$  F. Sixty milliliters of water are maintained in the tube, and oxygen is passed through the oil at the rate of 3 liters per hour. The test is continued until periodic testing shows that the oil has greatly increased in acidity, a sign of the formation of acidic oxidation products. These data are usually plotted graphically. Color can also be noted, although acidity is the primary criterion in this test.

In addition to the uninhibited base oil, four blends were subjected to this test. Blend R was a blend of 0.2 per cent, by weight, of N-[ $\beta$ -(anilino)-ethyl]-N'-phenylpiperazine (Example 1) in the base oil. Blend S comprised 0.2 per cent, by weight, of N-phenyl-N'-n-butylpiperazine (Example 4) in the base oil. Blend T comprised the base oil containing 0.2 per cent, by weight, of 4,4'-di[1-(4-n-butylpiperazino)]diphenylmethane (Example 5). Blend U was a blend of 0.2 per cent, by weight, of N,N'-di(p-t-amylphenyl)piperazine (Example 12) in the base oil. Pertinent test results for these blends are set forth in Table III.

Table III.—ASTM Turbine Oil Oxidation Test  
[(0.2% by weight of compound in base oil)]

| Example | Compound Tested                                   | Hours                            | Days                    | Color, Lovibond    | N. N.*               |
|---------|---------------------------------------------------|----------------------------------|-------------------------|--------------------|----------------------|
| 1.      | Uninhibited Base Oil                              | 24<br>48<br>72                   | 1<br>2<br>3             | 3<br>14<br>172     | 0.05<br>0.92<br>5.1  |
| 10.     | N-[ $\beta$ -(anilino)ethyl]-N'-phenylpiperazine. | 1,008<br>1,888<br>1,912          | 42<br>78<br>79          | 1.4<br>17<br>24    | 0.02<br>1.6<br>2.2   |
| 4.      | N-phenyl-N'-n-butylpiperazine.                    | 264<br>1,008<br>1,176            | 11<br>42<br>49          | 0.5<br>0.65<br>185 | 0.05<br>0.02<br>16.8 |
| 15.     | 4,4'-di[1-(4-n-butylpiperazino)]diphenylmethane.  | 1,920<br>2,952<br>3,624<br>3,728 | 80<br>123<br>151<br>155 | 2<br>3<br>7<br>260 | 0.06<br>0.60<br>10.7 |
| 5.      | N,N'-di(p-t-amylphenyl)piperazine.                | 72<br>144                        | 3<br>6                  | 8<br>330           | 0.8<br>10.6          |

\* Neutralization number.

In Figure 1, the acidity (N.N.) data for the tests reported in Table III are plotted graphically. As will be apparent from the curve for the base oil (curve A), uninhibited oils rapidly undergo oxidation. Curve A is a typical curve, in that the acidity remains low until oxidation commences. At that point, acidity increases rapidly, often within a matter of a few hours, causing a sharp rise in the curve. It will be noted that blend R maintained a low acidity throughout more than 42 days. It was not until almost 80 days had passed that the acidity increased. Test blend S lasted for about 49 days before acidity increased. In the case of blend T, the acidity remained low for about 150 days, and did not rise tremendously until about 5 days later. As compared with the foregoing, blend U lasted only 6 days on the ASTM Oxidation Test, indicating that the oxidation inhibition was very insignificant. It will be noted that this blend did not last much longer than the uninhibited base oil.

In the foregoing examples, the effectiveness of the compounds contemplated herein has been demonstrated. It will be appreciated that this relatively narrow class of substituted piperazine compounds is effective, when added to lubricating oils in small amounts, in inhibiting the oxidation thereof. It should be noted that when the compound has an aryl group directly attached to one nitrogen atom of the piperazine nucleus, the other nitrogen atom must have an alkyl group attached thereto. This can be appreciated by comparing the compounds of Examples 3 and 4 with the compounds of Examples 11 and 12.

Other oil addition agents can be used along with the additives of this invention, to improve other characteristics of the oil. For example, antirust agents, oiliness agents, E. P. agents, V. I. improvers, pour point depressants, detergents, antifoamants, and the like can be added to the mineral lubricating oil along with the additives of this invention. Such other additives are well known to those familiar with the art. Accordingly, it is believed unnecessary to list them here.

Although the present invention has been described in conjunction with preferred embodiments, modifications and variations are contemplated, as those skilled in the art will readily understand. Such variations and modifications are considered to be within the purview and scope of the appended claims.

What is claimed is:

1. A solvent-refined mineral steam turbine lubricating oil containing a small amount, sufficient to stabilize it against oxidation, of a com-

compound selected from the group consisting of (1) compounds having the formula,



wherein R is a radical of the group consisting of  $\beta$ -(phenylamino)ethyl,  $\beta$ -(naphthylamino)ethyl,  $\beta$ -(o-tolylamino)ethyl, and  $\beta$ -(m-tolylamino)ethyl radicals, and Y is a radical of the group consisting of phenyl, naphthyl, o-tolyl, and m-tolyl radicals; and (2) compounds having the formula,



wherein  $\text{R}''$  is an alkyl radical having between one and 8 carbon atoms, and  $\text{R}'$  is a radical of the group consisting of phenyl and naphthyl radicals and the radical having the formula,



2. A solvent-refined mineral steam turbine lubricating oil containing between about 0.05 per cent by weight and about 5 per cent by weight of a compound selected from the group consisting of (1) compounds having the formula,



wherein R is a radical of the group consisting of  $\beta$ -(phenylamino)ethyl,  $\beta$ -(naphthylamino)ethyl,  $\beta$ -(o-tolylamino)ethyl, and  $\beta$ -(m-tolylamino)ethyl radicals, and Y is a radical of the group consisting of phenyl, naphthyl, o-tolyl, and

m-tolyl radicals; and (2) compounds having the formula,



wherein  $\text{R}''$  is an alkyl radical having between one and 8 carbon atoms, and  $\text{R}'$  is a radical of the group consisting of phenyl and naphthyl radicals and the radical having the formula,



15 3. A solvent-refined mineral steam turbine lubricating oil containing a small amount, sufficient to stabilize it against oxidation, of  $\text{N}-[\beta$ -(anilino)-ethyl]- $\text{N}'$ -phenylpiperazine.

20 4. A solvent-refined mineral steam turbine lubricating oil containing a small amount, sufficient to stabilize it against oxidation, of  $\text{N}-[\beta$ -(1-naphthylamino)ethyl]- $\text{N}'$ -(1-naphthyl)piperazine.

25 5. A solvent-refined mineral steam turbine lubricating oil containing a small amount, sufficient to stabilize it against oxidation, of  $\text{N}$ -(1-naphthyl)- $\text{N}'$ -n-butylpiperazine.

30 6. A solvent-refined mineral steam turbine lubricating oil containing a small amount, sufficient to stabilize it against oxidation, of  $\text{N}$ -phenyl- $\text{N}'$ -n-butylpiperazine.

35 7. A solvent-refined mineral steam turbine lubricating oil containing a small amount, sufficient to stabilize it against oxidation, of 4,4'-di[1-(4-n-butylpiperazino)diphenylmethane].

References Cited in the file of this patent

UNITED STATES PATENTS

40 Number Name Date  
2,316,587 Irigai \_\_\_\_\_ Apr. 13, 1943